

## UNITED STATES PATENT OFFICE

2,189,054

## CASTING ZINC ALLOY

Arthur Burkhardt, Berlin-Lichterfelde, Germany,  
assignor to Georg Von Giesche's Erben, Breslau,  
Germany, a corporation of Germany

No Drawing. Application October 7, 1938, Serial  
No. 233,750. In Germany October 23, 1937

## 4 Claims. (Cl. 75—178)

My invention relates to zinc alloys containing aluminium and copper.

In my co-pending application, Ser. No. 170,853, for "Plastic zinc alloy", filed October 25, 1937, I have described a zinc alloy to which plasticity, i. e., good forging and extruding properties in cold condition, is imparted by providing a copper content of 2 to 8%, and by so determining the content of aluminium that it corresponds to the proportion of 12 to 22 parts of copper to 1 part of aluminium. In this manner, an alloy is obtained which possesses an unequalled constancy of dimensions.

It is an object of my present invention to provide a casting zinc alloy of constant dimensions.

As described in the said co-pending application, aluminium reduces and copper increases the length of casting alloys of this kind. This is due to the fact that casting alloys, as compared with cold-forged plastic alloys, do not possess a directional structure or anisotropic texture, but consist of irregularly distributed crystal grains. The changes in length produced by the aluminium and the copper are quite different and of a vectorial character. Another distinction as compared with the said plastic alloys is that changes of dimensions occur at a different velocity in plastic and in casting alloys.

Under these conditions, it was necessary to investigate proper proportions for an alloy which possesses good casting properties, and constant dimensions.

I have found that such an alloy comprises copper from 1 to 10%, aluminium from about 0.05 to about 0.6%, and zinc as the remainder, and that the copper and the aluminium must be proportioned at the rate of 17 to 19 parts of copper and 1 part of aluminium.

Alloys according to the invention, in addition to their good casting properties, possess considerable strength and are particularly suitable for gravity and pressure die casting. For instance, an alloy according to the invention possesses a tensile strength of over 27 kilogrammes per sq. millimeter, as compared with 13 to 17 kg./sq. mm. in alloys with tin or lead as the base, and constant dimensions, in pressure-die cast condition.

The remainder is zinc, preferably fine zinc, i. e., zinc of a high degree of purity, not less than 99.99%. However, the remainder may also be fine zinc with additions and impurities, for instance, with the addition of magnesium, as is usual in such zinc alloys. It is understood, there-

fore, that the phrase "the remainder being substantially all zinc" is intended to include fine zinc, particularly zinc of the aforesaid high degree of purity, and zinc containing minor amounts of additions or impurities which are usual in zinc alloys and do not influence the casting and other properties of the alloy according to my invention.

The following table gives examples of alloys according to the invention. In all cases, the balance is substantially zinc.

| Alloy No. | Copper, percent | Aluminium, percent | 15 |
|-----------|-----------------|--------------------|----|
| 1         | 2               | 0.111              |    |
| 2         | 3               | 0.166              |    |
| 3         | 4               | 0.222              |    |
| 4         | 5               | 0.278              |    |
| 5         | 6               | 0.333              |    |
| 6         | 7               | 0.389              |    |
| 7         | 8               | 0.444              | 20 |
| 8         | 9               | 0.5                |    |

The proportion of copper and aluminium is preferably 18 parts of copper to 1 part of aluminium, and the most favorable percentage of copper is about 4%. The proportion of 18:1 and the content of 4% copper are present in alloy No. 3, and it has been found that this alloy, in addition to its other favorable properties, possesses a high degree of constancy of dimensions in cast condition.

## I claim:

1. A casting zinc alloy of constant dimensions, comprising copper from 1 to 10%, aluminium from about 0.05 to about 0.6%, and the remainder being substantially all zinc; the copper and the aluminium being proportioned at the rate of 17 to 19 parts of copper and 1 part of aluminium.

2. A casting zinc alloy of constant dimensions, comprising copper from 1 to 10%, aluminium from about 0.05 to about 0.56%, and the remainder being substantially all zinc; the copper and the aluminium being proportioned at the rate of 18 parts of copper to 1 part of aluminium.

3. A casting zinc alloy of constant dimensions, comprising copper at the rate of about 4%, aluminium from about 0.21% to about 0.24%, and the remainder being substantially all zinc.

4. A casting zinc alloy of constant dimensions, comprising copper at the rate of about 4%, aluminium at the rate of about 0.222%, and the remainder being substantially all zinc.

ARTHUR BURKHARDT.